

## UNITED STATES PATENT OFFICE

ALBERT LOEBEL, OF AMSTERDAM, NETHERLANDS, ASSIGNOR TO DE BATAAFSCHE PETROLEUM MAATSCHAPPIJ, OF THE HAGUE, NETHERLANDS

## PROCESS FOR THE MANUFACTURE OF ASPHALT

No Drawing. Application filed February 14, 1929, Serial No. 340,006, and in the Netherlands December 9, 1927.

It is known that crude asphaltic oil, after any gasoline, kerosene and gasoil contained therein have been removed by distillation, yields on further distillation a residue which, depending on the extent to which the distillation is carried out, represents a more or less hard asphalt.

For practical purposes, asphalt should comply with various requirements which differ according to the purpose for which it is used. From a definite crude oil, only one and the same quality of asphalt may be obtained by distillation, which can only be modified slightly by altering the conditions under which the distillation takes place.

Also, with the aid of oxidizing treatments (the well-known blowing of asphalt), it is only possible to alter the quality of the asphalt gradually.

I have found, however, that the quality of the final product to be obtained from an oil may be highly improved by adding thereto, at any stage of the distillation (if desired, even to the starting material, i. e., the crude oil), at least 20% or more of hydrocarbons which are soluble in liquid  $\text{SO}_2$ , and my invention, broadly speaking, relates to such process. This material is obtained by extraction with liquid sulphur dioxide at a low temperature of liquid hydrocarbons with an initial boiling point of at least  $250^\circ \text{C}$ . The resulting extracts are mainly of an unsaturated character (aromatics are here taken also as unsaturated hydrocarbons).

If, according to my invention, an oil to which the said material is added, is subjected to a distillation with steam, a final product is obtained which is very tough in comparison with the product obtained from the same oil and under the same circumstances but without the addition of at least 20% of  $\text{SO}_2$ -soluble hydrocarbons.

Thus, if an oil yields, on distillation, a final product which is insufficiently tough or ductile—which, according to hitherto-known

methods, may be only improved to a certain extent by admixing other asphalts after distillation—I may add to that oil the above-mentioned material and then apply a distillation treatment with steam to the mixture in order to obtain an improved product.

If, according to my invention, an oil to which the said material is added, is subjected to an oxidizing distillation process, a final product is obtained which is very hard in comparison with the product obtained from the same oil and under the same circumstances but without the addition of at least 20 per cent of  $\text{SO}_2$ -soluble hydrocarbons. Thus, if an oil yields, on oxidizing distillation, a final product which is insufficiently hard, I may add to that oil the above-mentioned material and then apply an oxidizing distillation treatment to the mixture in order to obtain an improved product.

When speaking in the above of a "tough" or "ductile" asphalt, I mean that the consistency of such asphalt is sensitive to changes in temperature; that is to say, in terms well understood by those skilled in the art, its penetration curve is steep.

When speaking of a "hard" asphalt, I mean that its penetration curve is rather flat.

The following table contains some results obtained when applying my invention to Venezuelan residue:

| Steam asphalt         |                  | With the addition of 30 per cent $\text{SO}_2$ -soluble hydrocarbons | 80 |
|-----------------------|------------------|----------------------------------------------------------------------|----|
|                       | Without addition |                                                                      |    |
| Melting point (R & B) |                  |                                                                      |    |
| ASTM, D. 36-26        | 60° C.           | 61.5° C.                                                             | 85 |
| Penetration ASTM,     |                  |                                                                      |    |
| D. 5-25. at 0° C.     | 4                | 5                                                                    |    |
| at 15° C.             | 15               | 21                                                                   |    |
| at 25° C.             | 35               | 88                                                                   |    |
| Ductility ASTM,       |                  |                                                                      |    |
| D. 113-26 T. at 0° C. | 0                | 5                                                                    |    |
| at 15° C.             | 23               | 100                                                                  |    |
| at 25° C.             | 100              | 100                                                                  | 90 |

## Blown asphalt

|                      | Without addition | With the addition of 30 per cent $SO_2$ soluble hydrocarbons |
|----------------------|------------------|--------------------------------------------------------------|
| 5                    |                  |                                                              |
| 10                   |                  |                                                              |
| Melting point        | 128° C.          | 128° C.                                                      |
| Penetration at 0° C. | 6                | 4                                                            |
| at 15° C.            | 12               | 7.5                                                          |
| at 25° C.            | 20               | 13                                                           |
| at 40° C.            | 35               | 26                                                           |
| at 75° C.            | 121              | 82                                                           |

Finally, asphalts of entirely different specifications may be produced even from one single base material, for instance, by mixing with a fresh charge of the original base material the constituents which can be extracted from the distillates with liquid  $SO_2$ , this mixture being used for the manufacture of the asphalt.

What I claim is:

1. A process of manufacturing asphalt from crude oil, petroleum fractions, or petroleum residues, comprising the steps of adding to the initial material at least 20% of a hydrocarbon oil consisting of hydrocarbons soluble in liquid sulphur dioxide and having an initial boiling point of at least 250° C., and thereafter distilling the mixture in the presence of air to obtain an asphalt having a penetration curve flatter than that of an asphalt obtained without the addition of the hydrocarbon oil.
2. A process of manufacturing asphalt from crude asphaltic oil or asphaltic petroleum residues, comprising the steps of adding to the initial material a hydrocarbon oil extracted with liquid sulphur dioxide from petroleum distillates of the initial material and which hydrocarbon oil has an initial boiling point of at least 250° C., and thereafter distilling the mixture to produce an asphalt.
3. A process of manufacturing asphalt from crude asphaltic oil or asphaltic petroleum residues, comprising the steps of adding to the initial material at least 20% of extracted hydrocarbons soluble in liquid sulphur dioxide and having an initial boiling point of at least 250° C., and thereafter distilling the mixture with steam to obtain an asphalt which is more ductile and which has a penetration curve steeper than that of an asphalt obtained without the addition of the hydrocarbons.
4. A process of manufacturing asphalt from crude asphaltic oil or asphaltic petroleum residues, comprising the steps of adding to the initial material at least 20% of hydrocarbons, the total added hydrocarbons being substantially entirely soluble in liquid sulphur dioxide and having an initial boiling point of at least 250° C., and thereafter distilling the mixture with steam to obtain an asphalt which is more ductile and which has

a penetration curve steeper than that of an asphalt obtained without the addition of the hydrocarbons.

In testimony whereof I have affixed my signature.

ALBERT LOEBEL.

70

75

80

85

90

95

100

105

110

115

120

125

130